

May 26, 1953

F. PASSAL

2,640,021

COMPOSITION, BATH, AND PROCESS FOR CHROMIUM PLATING

Filed Nov. 23, 1949



Fig. 1

BATH AT 130°F (APPROX. 54.5°C)

Fig. 2  
BATH AT 110°F (43.3°C)



Fig. 3

BATH AT 90°F (APPROX. 32.2°C)

INVENTOR.

FRANK PASSAL

BY  
*G. R. Thompson*

## UNITED STATES PATENT OFFICE

2,640,021

COMPOSITION, BATH, AND PROCESS FOR  
CHROMIUM PLATINGFrank Passal, Detroit, Mich., assignor to United  
Chromium, Incorporated, New York, N. Y., a  
corporation of Delaware

Application November 23, 1949, Serial No. 129,128

14-Claims. (Cl. 204—51)

1

This invention relates to a chromium plating bath having exceptional plating performance and a self-regulated catalyst acid radical content, to compositions for making up such baths and to a chromium plating process and provides improvements therein.

It has heretofore been proposed to provide chromium plating baths in which the catalyst acid radical content is self-maintained or regulated with relation to a given chromic acid concentration, to provide a ratio of  $\text{CrO}_3$  to catalyst acid radical which gives satisfactory commercial chromium plating. Particular reference is made to the Lukens Patent No. 2,042,611. A sparingly soluble sulphate compound ( $\text{SrSO}_4$ ) is known from said patent, which will give  $\text{CrO}_3$  to  $\text{SO}_4$  ratios of approximately 100 to 1 with solutions of about 200 g./l. chromic acid. Most commercial chromium plating solutions have a chromic acid content higher than 200 g./l., commonly up to 400 to 500 g./l. No means has been heretofore discovered of providing for the self-regulation of the catalyst-acid radical content of commercially usable bath solutions containing the higher concentrations of chromic acid, such as 250 g./l. to 500 g./l.

According to the present invention, an aqueous chromium plating bath (and a composition for making up such a bath) is provided, which has a catalyst acid radical content supplied from strontium sulphate and potassium silicofluoride, these two compounds being present in excess of their solubilities in the bath, and which has a wide range of chromic acid concentrations, said bath giving superior performance, and being self-regulating as to the catalyst acid radical content in solution.

This invention also provides a chromium plating process, using modes of procedure in baths according to the present invention for attaining (1) fast deposition of thick, good quality bright chromium plate, (2) fast deposition of thick, good quality gray chromium plate, and (3) high covering power in the deposition of bright chromium plate in usual decorative plate thicknesses.

The bath (aqueous) essentially consists of about 200 to 500 g./l.  $\text{CrO}_3$ , strontium sulphate ( $\text{SrSO}_4$ ) present in excess of its solubility in the chromic acid solution and potassium silicofluoride ( $\text{K}_2\text{SiF}_6$ ) also present in excess of its solubility in the chromic acid solution.

The use of chromic acid of high purity is recommended, such as chromic acid containing less than 0.1% by weight of sulphate and no other catalyst acid radicals. Chromic acid or

2

higher sulphate content can be used by first analysing for  $\text{SO}_4$  and then adding approximately the stoichiometric equivalent of strontium carbonate to form  $\text{SrSO}_4$  with the  $\text{SO}_4$  impurity, or by adding the stoichiometric equivalent of barium carbonate, barium hydroxide, or barium chromate for the  $\text{SO}_4$  in the chromic acid.

Either a C. P. (chemically pure) or a good technical grade of strontium sulphate may be used. One form of strontium sulphate commercially available is the mineral Celestite which may be also used satisfactorily.

Either C. P. (chemically pure) or a good technical grade of  $\text{K}_2\text{SiF}_6$  can be used.

15 The  $\text{SrSO}_4$  and  $\text{K}_2\text{SiF}_6$  instead of being added as such to the composition of matter or to the bath, may be added in the form of non-catalytic strontium and potassium compounds and  $\text{SO}_4$  and  $\text{SiF}_6$  compounds which will interact in solution to form  $\text{SrSO}_4$  and  $\text{K}_2\text{SiF}_6$  in amounts which will more than saturate the solutions and provide an undissolved excess or reservoir of  $\text{SrSO}_4$  and  $\text{K}_2\text{SiF}_6$  from which  $\text{SO}_4$  and  $\text{SiF}_6$  catalyst acid radicals lost from the bath in the course of operation will be replenished.

20 Examples of non-catalytic strontium and potassium compounds are  $\text{SrCO}_3$ ,  $\text{Sr}(\text{OH})_2$ ,  $\text{SrCrO}_4$ , etc. and  $\text{KOH}$ ,  $\text{K}_2\text{CO}_3$ ,  $\text{K}_2\text{CrO}_4$ ,  $\text{K}_2\text{Cr}_2\text{O}_7$ . Examples of suitable  $\text{SO}_4$  and  $\text{SiF}_6$  compounds referred to above are  $\text{H}_2\text{SO}_4$ ,  $\text{Na}_2\text{SO}_4$ ,  $\text{Li}_2\text{SO}_4$ ,  $(\text{NH}_4)_2\text{SO}_4$ , 30  $\text{CaSO}_4$ , etc. and  $\text{H}_2\text{SiF}_6$ ,  $\text{NaSiF}_6$ ,  $(\text{NH}_4)_2\text{SiF}_6$ ,  $\text{MgSiF}_6$ ,  $\text{CaSiF}_6$ , etc.

25 A solid composition of matter may be therefore prepared comprising  $\text{CrO}_3$ ,  $\text{SrSO}_4$  and  $\text{K}_2\text{SiF}_6$  as such, or by adding  $\text{CrO}_3$ , and a suitable strontium compound, a suitable sulphate compound, a suitable potassium compound and a suitable silicofluoride compound as suggested above. On adding both types of composition of matter to water to give  $\text{CrO}_3$  concentrations within the range 200 to 500 g./l., the end-result will be the same.

30 The composition consists of chromic acid and enough  $\text{SrSO}_4$  and  $\text{K}_2\text{SiF}_6$  to provide as a minimum an undissolved excess of  $\text{SrSO}_4$  and  $\text{K}_2\text{SiF}_6$  at any desired bath concentration within the 45  $\text{CrO}_3$  range of concentration, and at any desired temperature within the operating range of temperature.

Examples of compositions are as follows:

50

Example I

|                                    | Parts by weight |
|------------------------------------|-----------------|
| $\text{CrO}_3$ , 97.7%             | 100             |
| $\text{SrSO}_4$ , 0.6%             | 0.61            |
| 55 $\text{K}_2\text{SiF}_6$ , 1.7% | 1.74            |

The above composition will provide a bath solution saturated at 90° F. with  $\text{SrSO}_4$  and  $\text{K}_2\text{SiF}_6$  using this composition of matter in water to give  $\text{CrO}_3$  concentrations of or near 500 g./l.

*Example II*

|                                 | Parts by weight |
|---------------------------------|-----------------|
| $\text{CrO}_3$ , 95.3%          | 100             |
| $\text{SrSO}_4$ , 1.4%          | 1.47            |
| $\text{K}_2\text{SiF}_6$ , 3.3% | 3.5             |

The above composition will provide a bath solution saturated at 90° F. with  $\text{SrSO}_4$  and  $\text{K}_2\text{SiF}_6$  at minimum  $\text{CrO}_3$  concentration (200 g./l.), and an excess of  $\text{SrSO}_4$  and  $\text{K}_2\text{SiF}_6$  at higher  $\text{CrO}_3$  concentrations, using this composition of matter.

*Example III*

|                                 | Parts by weight |
|---------------------------------|-----------------|
| $\text{CrO}_3$ , 90.1%          | 100             |
| $\text{SrSO}_4$ , 2.7%          | 3               |
| $\text{K}_2\text{SiF}_6$ , 7.2% | 8               |

The above composition will give a bath saturated with  $\text{SrSO}_4$  and  $\text{K}_2\text{SiF}_6$ , together with an undissolved excess, at any  $\text{CrO}_3$  concentration within the range 200 to 500 g./l., using this composition of matter. This composition, from the practical standpoint, also provides  $\text{SrSO}_4$  and  $\text{K}_2\text{SiF}_6$  in sufficient excess to hasten saturation equilibrium in initial bath makeup, and to insure always having present an undissolved excess. Obviously there is no theoretical upper limit to the quantities of  $\text{SrSO}_4$  and  $\text{K}_2\text{SiF}_6$  that can be used.

*Example IV*

|                                 | Parts by weight |
|---------------------------------|-----------------|
| $\text{CrO}_3$ , 92.5%          | 100             |
| $\text{SrSO}_4$ , 2.0%          | 2.16            |
| $\text{K}_2\text{SiF}_6$ , 5.5% | 5.95            |

A single composition, as Example III, has the advantage of having universal suitability throughout the full range of  $\text{CrO}_3$  concentration, but the composition such as Example II having lesser percentages of  $\text{SrSO}_4$  and  $\text{K}_2\text{SiF}_6$  also are suitable for bath solutions of higher  $\text{CrO}_3$  content. Example I represents the minimum percentages of  $\text{SrSO}_4$  and  $\text{K}_2\text{SiF}_6$  usable at the maximum  $\text{CrO}_3$  concentration and hence the minimum percentage which can be used and still be within the range of  $\text{CrO}_3$  bath concentrations herein disclosed. Example IV represents a composition in commercial use.

This bath makeup has a much higher degree of flexibility than any previously known chromium plating bath as regards the relationship of the catalyst acid radicals to the chromic acid content, and in addition the bath is self-regulating.

There is a great advantage in the self-regulating feature of the present bath by its obviating need for analytical determination of silicofluoride content, in that analyses for silicofluoride in chromic acid are very difficult to make.

The effect of the silicofluoride in the bath does not appear to be in arithmetic progression (additive) in relation to quantity added; that is, the catalytic effect of the  $\text{SiF}_6$  in the present bath was found to have no definite or predictable effect by analogy to  $\text{CrO}_3/\text{SO}_4$  current efficiency curves. The effect of the silicofluoride also appears to be affected by the amount of  $\text{SO}_4$  present, the amount of  $\text{CrO}_3$  and the temperature of the bath.

Chromium plating baths containing silicofluoride went into considerable use some fifteen years ago, but have largely gone out of use, due probably to the difficulty of analysing them, the dif-

fulness of maintaining uniform operating characteristics, and to the fact that deposits other than very thin deposits were pimply. The deposits obtained by the use of the present invention

are not pimply. The deposits are smooth at all  $\text{CrO}_3$  concentrations, have little or no tendency to "tree" at high plating speeds and have leveling action. Deposits over about one-half thousandth of an inch from baths containing from 400 to 500 g./l.  $\text{CrO}_3$  have a matte appearance, and are exceptionally smooth and free from nodules. Deposits in decorative plate thicknesses are bright throughout the  $\text{CrO}_3$  concentration range.

The performance of baths according to the present invention is exceptional, and not in accordance with what had been expected from conventional ideas as to the effect of the  $\text{CrO}_3$ /total catalyst acid radical ratio.

In contrast with the generally used  $\text{CrO}_3/\text{SO}_4$  chromium plating bath, a bath according to the present invention containing  $\text{SrSO}_4$  and  $\text{K}_2\text{SiF}_6$  present in excess of the solubilities thereof in the bath can vary over a wide range of  $\text{CrO}_3$  concentrations, ranging from about 200 g./l. to 500 g./l., with neither a wide nor a significant variation in the current efficiencies at commonly used temperatures over a wide range of current densities (1-6 amperes per square inch at 130° F. for instance). Moreover, the current efficiencies of baths within the present invention are generally higher than the best current efficiencies obtainable with the  $\text{CrO}_3/\text{SO}_4$  baths; and, within the  $\text{CrO}_3$  range, and, at separate parts of the  $\text{CrO}_3$  range, are found baths having superior performance in differing particulars. Baths having optimum throwing power are obtained with a  $\text{CrO}_3$  content of about 450 g./l., with excellent throwing power at 400 to 500 g./l.  $\text{CrO}_3$ . For barrel plating a 450 g./l.  $\text{CrO}_3$  concentration has been found to give optimum performance.

Baths containing from about 250 g./l. to 350 g./l.  $\text{CrO}_3$ , with optimum at about 325 g./l.  $\text{CrO}_3$ , have been found to give the highest current efficiencies and highest plating speeds, and bright deposits in heavy thicknesses. The 250 to 350 g./l.  $\text{CrO}_3$  range is recommended for so called "hard chromium" plating, where plating speed is of great importance and bright deposits in heavy thickness are desired. High plating speed results from high current efficiency, and the feasible use of higher current densities. As compared with the conventional  $\text{CrO}_3/\text{SO}_4$  bath, the bath of the present invention within the 250 to 350  $\text{CrO}_3$  range (optimum 325 g./l.  $\text{CrO}_3$ ) has the advantage of considerably higher current efficiency and less tendency for treeing and has leveling action.

The current efficiencies of aqueous baths containing 200 g./l. to 500 g./l.  $\text{CrO}_3$  saturated with  $\text{SrSO}_4$  and  $\text{K}_2\text{SiF}_6$  at 130° F. (54.4° C.), 110° F. (43.3° C.) and 90° F. (32.2° C.) for representative ranges of current densities are shown in the graphs, Figs. 1, 2 and 3. Current efficiencies for baths containing more than 350 g./l.  $\text{CrO}_3$  are still excellent; but above 350 g./l. the deposits in thicknesses above about 0.0001" range, in appearance, from satiny semi-bright to full dull gray matte and, in texture, remain unusually smooth and velvety. Although bright deposits are generally preferred for so called "hard" or industrial chromium plate, this gray matte deposit is an excellent plate, and, as with the bright deposits, is extremely smooth, exhibiting definite "leveling action" of surface scratches or

defects, as determined by profilometer measurements, and as contrasted with deposits produced in the conventional bath. The deposit also has a minimum tendency to formation of nodules and "trees." In addition these deposits have been found to be harder (by scratch hardness tests, using the Bierbaum microcharacter) than corresponding bright deposits from the conventional  $\text{CrO}_3/\text{SO}_4$  bath.

The brightness of the deposits, the smoothness of the deposits, the covering power and the current efficiency obtained from baths according to the present invention are superior to those from the standard  $\text{CrO}_3/\text{SO}_4$  bath. The baths also have a broader bright plating range than the standard  $\text{CrO}_3/\text{SO}_4$  bath, and are especially suitable for plating bright directly on stainless steel and zinc base die-castings.

Another advantage of the present baths is that if a bright nickel surface is passive, or otherwise not receptive to a good chromium deposit, or if the current density is too low for complete coverage, an iridescent oxide, or oxide-chromate film commonly obtained with the conventional  $\text{CrO}_3/\text{SO}_4$  bath will not be left on the areas not covered by the chromium. A partly chromium covered nickel plated part plated in the present bath can have the chromium stripped from it and be replated with chromium without the necessity of re-buffering the nickel before replating with chromium. A partly chromium covered nickel plated part plated in the ordinary chromic acid-sulphate bath would have an iridescent oxide or oxide-chromate film on the uncovered parts, and the parts covered by the film would be etched in stripping the chromium, and re-buffering would be required before replating with chromium.

The present baths give chromium deposits which are less sensitive to interruption of current, which in the chromic acid-sulphate bath ordinarily causes objectionable gray deposits or poor adhesion; and have a better activating action on nickel plate than the usual chromic acid-sulphate bath.

The process for the fast deposition of thick, good quality, bright chromium plate is carried out as follows: The plating bath is one according to this invention having a  $\text{CrO}_3$  concentration of 200 to 350 g./l. (325 g./l. optimum). Thick bright deposits (0.001" or more by way of example) may be electroplated at current densities and bath temperatures generally used for chromium deposition (see Modern Electroplating, The Electrochemical Society, 1942, chapter on Chromium Plating, and particularly the charts on pages 122 and 123). The higher temperatures and current densities are usually employed for obtaining thick deposits; and such are best used in the present process for rapidly obtaining thick deposits, the advantage here being that current efficiencies better than are obtained in the conventional  $\text{CrO}_3/\text{SO}_4$  bath are obtained, and higher current densities can be used without a rough or "treed" plate being obtained. Figure 1 shows the relatively high current efficiencies which can be obtained at 1-6 amperes per square inch, temperature 130° F. (about 55° C.), particularly in a bath with a  $\text{CrO}_3$  concentration of about 325 g./l.

The process for the fast deposition of thick, good quality semi-bright to gray chromium plate is carried out as follows:

The plating bath is one according to this invention having  $\text{CrO}_3$  concentrations of 350 to 500 g./l. (425 g./l. optimum). Thick gray deposits

(0.001" or more by way of example) may be electroplated at current densities and bath temperatures generally used for chromium deposition (see Modern Electroplating referred to above). The higher temperatures and current densities are usually employed for obtaining thick deposits; and such are best used in the present process for rapidly obtaining thick deposits, the advantage here being that the current efficiencies are better than those obtained by the conventional  $\text{CrO}_3/\text{SO}_4$  baths and higher current densities can be used without a rough or "treed" plate being obtained. In fact the thick gray chromium deposits are especially smooth and free from nodules. Where chromium plate must be ground or otherwise finished for dimensional requirements or fit, deposits such as are produced by the present process are particularly advantageous. Figure 1 shows the relatively high current efficiencies which can be obtained at 1-6 amperes per square inch, temperature 130° F. (about 55° C.), particularly in a bath with a  $\text{CrO}_3$  concentration of about 350 to 500 g./l.

The process for attaining high covering power in the deposition of bright chromium plate, in usual decorative plate, is carried out as follows:

The plating bath is one according to the invention, having a  $\text{CrO}_3$  concentration of 350 to 500 g./l. (400 to 500 g./l. optimum). The deposits are the kind used for so called decorative bright plate and commonly are a few hundredths thousandths inch thick. These decorative bright deposits may be electroplated at current densities and bath temperatures generally used for chromium deposition (see Modern Electroplating, referred to above). Speed of plating usually not being as important for decorative plate as for thick so called hard chromium plate, a considerable choice of temperatures and current densities is available. Figures 1, 2 and 3 show examples of temperatures and current densities for use. The curves for the lowest current densities in these three figures are indicative of the better covering power of the solutions at the higher chromic acid concentrations. The chromium plate obtained is unusually bright.

The process for attaining a bright deposit in a chromium plating barrel is carried out as follows:

The plating bath is one according to the invention having a  $\text{CrO}_3$  concentration of 450 g./l. as optimum. The bright deposits are electroplated at current densities and bath temperatures generally used for chromium deposition in barrels. A temperature in the neighborhood of 90° F. is often used for barrel plating. The temperature and current density of the bath, to some extent, depends on the work being plated, the temperature and current density being always fixed at those that give the best coverage.

This application is a continuation in part of application Serial No. 69,534, filed January 6, 1949, now abandoned.

What is claimed is:

1. A composition of matter for making up an aqueous chromium plating bath comprising essentially chromic acid, strontium sulphate and potassium silicofluoride, there being about 3 parts by weight of strontium sulphate and about 8 parts by weight potassium silicofluoride to 100 parts by weight chromic acid, said composition when dissolved in water being adapted to produce a solution having a concentration of 200 to 500 g./l. chromic acid.

2. A composition of matter for making up an

aqueous chromium plating bath, comprising essentially chromic acid, strontium sulphate and potassium silicofluoride, there being about 2.16 parts by weight strontium sulphate and about 5.95 parts by weight potassium silicofluoride to 100 parts by weight chromic acid, said composition when dissolved in water being adapted to produce a solution having a concentration of 200 to 500 g./l. chromic acid.

3. An aqueous bath for chromium plating consisting essentially of 200 to 500 g./l. chromic acid, and strontium sulphate and potassium silicofluoride present each in amounts in excess of the solubility thereof in the chromic acid solution.

4. An aqueous bath for chromium plating consisting essentially of 400 to 500 g./l. chromic acid, and strontium sulphate and potassium silicofluoride present each in amounts in excess of the solubility thereof in the chromic acid solution.

5. An aqueous bath for chromium plating consisting essentially of 250 to 350 g./l. chromic acid, and strontium sulphate and potassium silicofluoride present each in amounts in excess of the solubility thereof in the chromic acid solution.

6. A process of electrodepositing chromium consisting essentially of passing current from an anode to an article-cathode immersed in a bath consisting essentially of 200 to 500 g./l. chromic acid and strontium sulphate and potassium silicofluoride present in the bath each in excess of its solubility therein.

7. A process of electrodepositing thick, bright chromium of good quality consisting essentially of passing current from an anode to an article-cathode immersed in a bath consisting essentially of 200 to 350 g./l.  $\text{CrO}_3$  and strontium sulphate and potassium silicofluoride present in the bath each in excess of its solubility therein.

8. A process of electrodepositing chromium of good quality consisting essentially of passing current from an anode to an article-cathode immersed in a bath consisting essentially of 350 to 500 g./l.  $\text{CrO}_3$  and strontium sulphate and potassium silicofluoride present in the bath each in excess of its solubility therein.

9. A process of electrodepositing bright chromium in plating barrels, consisting essentially of passing current from an anode to an article-cathode immersed in a bath consisting of 450 g./l.  $\text{CrO}_3$  and strontium sulphate and potassium silicofluoride present in the bath each in excess of its solubility therein.

10. A composition of matter for making up and maintaining aqueous baths for chromium plating comprising essentially chromic acid, strontium sulphate, and potassium silicofluoride, the strontium sulphate content being in excess of about 0.61 part by weight to 100 parts by weight of chromic acid and the potassium silicofluoride content being in excess of about 1.74 parts by weight to 100 parts by weight of chromic acid, said composition when dissolved in water to produce a solution having 200 to 500 g./l. of chromic acid dissolved therein, also producing in such solution dissolved amounts of strontium sulphate and potassium silicofluoride sufficient to saturate said solution, and also undissolved amounts of strontium sulphate and potassium silicofluoride.

11. A composition of matter for making up and maintaining aqueous baths for chromium plating comprising essentially chromic acid, strontium sulphate, and potassium silicofluoride, the

strontium sulphate content being in excess of about 0.61 part by weight to 100 parts by weight of chromic acid and the potassium silicofluoride content being in excess of about 1.74 parts by weight to 100 parts by weight of chromic acid, said composition when dissolved in water being adapted to produce a solution having excess undissolved amounts of strontium sulphate and potassium silicofluoride.

10. 12. A composition of matter for making up and maintaining aqueous baths for chromium plating comprising essentially chromic acid, strontium sulphate, and potassium silicofluoride, the strontium sulphate content being in excess of about 0.61 part by weight to 100 parts by weight of chromic acid and the potassium silicofluoride content being in excess of about 1.74 parts by weight to 100 parts by weight of chromic acid.

15. 13. A composition of matter for making up and maintaining an aqueous chromium plating bath comprising essentially chromic acid, strontium sulphate and potassium silicofluoride, there being at least about 1.47 parts by weight of strontium sulphate and at least about 3.5 parts by weight of potassium silicofluoride to 100 parts by weight of chromic acid, said composition when dissolved in water being adapted to produce a solution having a concentration of 200 to 500 g./l. of chromic acid.

20. 14. A composition of matter for making up and maintaining an aqueous chromium plating bath comprising essentially chromic acid, (1) a bath-soluble compound containing catalytic sulphate radical, (2) a bath-soluble strontium compound of a non-catalytic anion, the amount of said strontium compound being stoichiometrically equivalent to the amount of said sulphate compound so as to react therewith in said bath to form strontium sulphate, (3) a bath-soluble compound containing catalytic silicofluoride radical, and (4) a bath-soluble potassium compound of a non-catalytic anion, the amount of said potassium compound being stoichiometrically equivalent to the amount of said silicofluoride compound so as to react therewith in said bath to form potassium silicofluoride, the said four compounds being present in such quantities to form at least about 0.61 part by weight strontium sulphate to 100 parts by weight of chromic acid and at least about 1.74 parts by weight of potassium silicofluoride to 100 parts by weight of chromic acid, said composition when dissolved in water to produce a solution having 200 to 500 g./l. of chromic acid dissolved therein, also producing in such solution dissolved amounts of strontium sulphate and potassium silicofluoride sufficient to saturate said solution, and also undissolved amounts of strontium sulphate and potassium silicofluoride.

FRANK PASSAL.

References Cited in the file of this patent

UNITED STATES PATENTS

| Number       | Name              | Date           |
|--------------|-------------------|----------------|
| 65 1,815,081 | Sohn et al. ----- | July 21, 1931  |
| 1,844,751    | Fink et al. ----- | Feb. 9, 1932   |
| 1,864,014    | Ewing -----       | June 21, 1932  |
| 1,928,284    | Fink et al. ----- | Sept. 26, 1933 |
| 2,042,611    | Lukens -----      | June 2, 1936   |

70 FOREIGN PATENTS

| Number  | Country             | Date          |
|---------|---------------------|---------------|
| 566,218 | Great Britain ----- | Dec. 19, 1944 |